

# United States Patent Office

3,018,619

Patented Jan. 30, 1962

1

3.018.619

3,516,519

**MONOPROPELLANTS CONTAINING QUATERNARY AMMONIUM COMPOUNDS**

Richard C. Doss and William B. Reynolds, Bartlesville, Okla., assignors to Phillips Petroleum Company, a corporation of Delaware

No Drawing. Filed July 17, 1959, Ser. No. 827,976  
16 Claims. (Cl. 60—35.4)

This invention relates to monopropellant compositions suitable for use in rocket motors, ram-jets, pulse-jets and the like. In a further aspect, this invention relates to a method of operating such motors.

Rocket motors are operated by burning a mixture of fuel and oxidant in a combustion chamber thereof and causing the resulting gases to be expelled through a nozzle at high velocity. Liquid propellants are preferred over solid propellants where it is necessary to vary thrust during flight. Liquid propellants can be classified as bipropellants and monopropellants, and the latter can be either a single compound or mixtures of compounds. Monopropellant systems are advantageous in that they require only one tank, one pump, one nozzle, one fuel line, one set of controls, etc. Furthermore, no mixing or proportioning system is required.

The principal elements of a rocket motor utilizing a liquid fuel comprise a combustion chamber, exhaust nozzle, an injection system, and propellant control valves. The propellant gases are produced in the combustion chamber at pressures governed by the chemical characteristics of the propellant, its rate of consumption, and the cross-sectional area of the nozzle throat. The gases are ejected into the atmosphere through the nozzle with supersonic velocity. The function of the nozzle is to convert the pressure of the propellant gases into kinetic energy. The reaction of the discharge of the propellant gases constitute the thrust developed by the rocket motor.

The following are objects of this invention.

An object of this invention is to provide new monopropellant composition. A further object of this invention is to provide a method for operating rocket motors. Other aspects, objects and advantages of the invention will be apparent to those skilled in the art in view of this disclosure.

In accordance with the invention there are provided new monopropellant compositions which are suitable for use according to the method of the invention in rocket motors and the like. Broadly speaking, the invention comprises a mixture of a quaternary ammonium compound and a suitable oxidant as a monopropellant composition and the use of said composition as a propellant in a rocket motor or the like.

in a rocket motor of the like.

Thus according to the invention there is provided a monopropellant composition comprising a mixture of (1) an oxidant selected from the group consisting of nitric acid containing at least about 70 weight percent  $\text{HNO}_3$  and mixtures of said nitric acid with perchloric acid wherein said mixtures contain up to about 50 weight percent  $\text{HClO}_4$  and not more than about 30 weight percent water, and (2) at least one quaternary ammonium compound characterized by a formula selected from the group consisting of

and

2



10 wherein: each R is selected from the group consisting of alkyl, cycloalkyl, alkenyl, and cycloalkenyl radicals containing from 1 to 8 carbon atoms wherein when more than one carbon atom is present the carbon atom attached to the quaternary nitrogen atom is attached to adjoining carbon atoms by single valence bonds, and said radicals substituted with a substituent selected from the group consisting of nitro, nitroso, and cyano radicals, the total 15 number of said substituents in said R groups being not greater than one-half the total number of carbon atoms in said R groups; R' is selected from the group consisting of alkylene radicals containing from 1 to 12 carbon atoms, and alkenylene radicals containing from 4 to 12 20 carbon atoms wherein the carbon atoms attached to the quaternary nitrogen atom is attached to adjoining carbon atoms by a single valence bond; X is an anion selected from the group consisting of nitrate, perchlorate, mono-hydrogen phosphate, dihydrogen phosphate, hydrogen 25 sulfate, sulfate, hydroxyl, orthoborate, dihydrogen borate, and tetraborate anions; a and b are each integers of from 1 to 4, and the product of a multiplied by the number of quaternary nitrogen atoms is equal to the product of b multiplied by the valence of said anion X; and wherein 30 the ratio of said quaternary ammonium compound to said oxidant is within the range of 0.75 to 1.25 times that of the stoichiometric amount.

It is to be noted that the compounds used in the practice of the invention are quaternary ammonium compounds as distinguished from acid salts of amines. The two classes of compounds are distinctly different chemically. As used herein and in the claims the term "quaternary ammonium compound" refers to a compound containing at least one nuclear nitrogen atom having its five so-called valence bonds attached to atoms (or radicals) other than a hydrogen atom. For example, such as four nitrogen to carbon bonds and one nitrogen to nitrate (or other anionic radical) bond. In other words, the available valence bonds of said nuclear nitrogen atom are satisfied by other than a hydrogen radical. For example, consider the two compounds (1) trimethylamine nitrate and (2) tetramethyl ammonium nitrate which have the formulas  $(CH_3)_3NHNO_3$  and

50 respectively. It will be noted that in the acid salt trimethylamine nitrate one of the valence bonds of the nuclear nitrogen atom is satisfied by a hydrogen atom whereas in the quaternary ammonium compound tetra-  
 55 methyl ammonium nitrate all five valence bonds are satisfied by radicals other than hydrogen.

The two classes of compounds can also be distinguished by their reaction with strong bases. For example, when an acid salt such as trimethylamine nitrate is reacted with 60 sodium hydroxide the amine is liberated along with the formation of sodium nitrate and water; whereas a quaternary ammonium compound such as tetramethyl ammonium nitrate has no hydrogen available for the formation of water and there is obtained the tetramethyl ammonium hydroxide,  $(\text{CH}_3)_4\text{NOH}$  and sodium nitrate, and 65 no free amine is liberated.

As shown hereinafter the monopropellants of the invention using the above defined quaternary ammonium compounds are markedly more stable than monopropellants using acid salts of amines.

Examples of quaternary ammonium compounds suit-



able for use in the practice of the invention include, among others, the following:

Tetramethylammonium nitrate  
 Tetramethylammonium perchlorate  
 Tetramethylammonium hydrogen sulfate  
 Tetraethylammonium nitrate  
 Triethylmethylammonium hydrogen sulfate  
 Triethylmethylammonium nitrate  
 Triethylmethylammonium perchlorate  
 Triethylmethylammonium dihydrogenphosphate  
 Diethylmethylammonium nitrate  
 Ethyltrimethylammonium nitrate  
 Diallyldimethylammonium nitrate  
 Tetra-n-propylammonium nitrate  
 Tetra-n-propylammonium dihydrogen phosphate  
 Tetra-n-propylammonium hydrogen sulfate  
 Di(2-methylhexyl)dimethylammonium perchlorate  
 Tetra-n-butylammonium nitrate  
 Tetra-n-butylammonium perchlorate  
 Trimethylpentylammonium perchlorate  
 Ethyltritylammmonium perchlorate  
 Dihexyldi-n-propylammonium nitrate  
 Ethyltri-n-octylammonium nitrate  
 Tetra-n-octylammonium nitrate  
 Methyltri-n-octylammonium nitrate  
 Methyltri-tert-octylammonium nitrate  
 N,N,N',N'-tetramethyl diethylenediammonium dinitrate  
 N,N,N',N'-tetra-n-butyl diethylenediammonium dinitrate  
 Trimethylcyclohexylammonium nitrate  
 Trimethylcyclohexylammonium metaborate  
 Allyltrimethylammonium nitrate  
 Triethyl-2-methylallylammonium nitrate  
 3-hexenyltriethylammonium nitrate  
 Di-3-hexenyldimethylammonium nitrate  
 Ethyldimethyl-2-cyclooctenylammonium nitrate  
 Allyldiethylcyclohexylammonium perchlorate  
 N,N,N',N',N'-hexamethyl methanediammonium dinitrate  
 N,N,N',N',N'-hexamethyl methanediammonium diperchlorate  
 N,N,N',N',N'-hexaethyl methanediammonium diperchlorate  
 N,N,N',N',N'-hexamethylethane-1,2-diammonium dinitrate  
 N,N,N',N',N'-hexamethylpropane-1,3-diammonium dinitrate  
 N,N,N',N',N'-hexamethylbutane-1,4-diammonium dinitrate  
 N,N,N',N',N'-hexamethylbutane-1,4-diammonium diperchlorate  
 N,N,N',N',N'-hexamethylbutane-1,4-bis(diammonium hydrogen phosphate)  
 N,N,N',N',N'-hexamethylbutane-1,4-bis(ammonium hydrogen sulfate)  
 N,N,N',N',N'-hexa-n-propylbutane-1,4-diammonium dinitrate  
 N,N,N',N',N'-hexamethyloctane-1,8-diammonium dinitrate  
 N,N,N',N',N'-hexamethyldodecane-1,12-diammonium dinitrate  
 N,N,N',N',N'-hexa(2-nitroethyl)propane-1,3-diammonium dinitrate  
 N,N,N',N',N'-hexa(2-cyanoethyl)hexane-1,6-diammonium dinitrate  
 N,N,N',N',N'-hexa(2-cyanoethyl)hexane-1,4-diammonium dinitrate  
 N,N,N',N',N'-hexamethyl(2-butene)1,4-diammonium dinitrate  
 N,N'-dimethyltriethylene diammonium dinitrate  
 N,N'-dimethyltriethylene diammonium diperchlorate  
 N,N'-diethyltriethylene diammonium dinitrate  
 N-ethyl-N'-methyltriethylene diammonium dinitrate  
 N,N'-diisopropyltriethylene diammonium dinitrate  
 N,N'-dicyclohexyltriethylene diammonium dinitrate

N,N,N,N',N',N'-hexamethyl(4-dodecene)-1,12-diammonium dinitrate  
 N,N,N,N',N',N'-hexaethyl(2,7-diethyl-4-octene)-1,7-diammonium dinitrate  
 5 Tetramethyl ammonium tetraborate  
 Ethyltrimethyl ammonium orthoborate  
 Triethylmethyl ammonium perborate  
 Tetramethylammonium hydroxide  
 Tetraethylammonium hydroxide  
 10 Tetra-n-propylammonium hydroxide  
 Trimethylpentylammonium hydroxide  
 Methyltri-n-octylammonium hydroxide  
 N,N,N',N',N'-hexamethylmethane diammonium hydroxide  
 15 N,N,N',N',N'-hexaethyloctane-1,8-diammonium hydroxide

The quaternary ammonium compounds described above are oxygen deficient and consequently the monopropellant fuel compositions of my invention require an oxidant. 20 Nitric acid is the presently preferred oxidant for use in the practice of the invention. Since water tends to retard combustion of the acid with the fuel, the nitric acid is preferably substantially free of water. Thus, the presently most preferred oxidant is anhydrous nitric acid. 25 However, other more dilute nitric acids can be used in the practice of the invention. White fuming nitric acids and red fuming nitric acids of varying concentrations are available commercially, and all are useful in the practice of this invention. White fuming nitric acid usually 30 contains about 90 to 99 weight percent HNO<sub>3</sub>, from 0 to 2 weight percent NO<sub>2</sub>, and up to about 10 weight percent water. Red fuming nitric acid usually contains about 70 to 90 weight percent HNO<sub>3</sub>, from 2 to 25 weight percent NO<sub>2</sub>, and up to about 10 weight percent water. 35 Of course, mixtures of the above described acids can be employed to give an acid having any intermediate composition, and all are useful in the practice of this invention. Thus, it has been found that nitric acids of all types containing at least about 70 weight percent HNO<sub>3</sub> 40 are useful as an oxidant in the practice of the invention. In addition, it is within the scope of the invention to use mixtures of said nitric acid with perchloric acid wherein said mixtures contain up to about 50 weight percent HClO<sub>4</sub>. As an oxidant in the practice of the invention. Said mixtures preferably do not contain more than 45 about 30 weight per cent water.

The monopropellants used in the present invention will be preferably near stoichiometric mixtures of oxidant and quaternary ammonium compound. The ratio of fuel component to oxidant can be in the range of 0.75 to 1.25 times that of the stoichiometric amount. In the practice of the invention said quaternary compounds are commonly used in amounts of about 17 to about 48 weight percent of the mixture of oxidant and quaternary ammonium compound. A slightly fuel-rich mixture is usually required to give an optimum rocket motor performance. As used herein stoichiometric ratio is that ratio of fuel to oxidant calculated by assuming complete combustion of the nitrogen, hydrogen, and carbon of the fuel 60 to N<sub>2</sub>, H<sub>2</sub>O, and CO<sub>2</sub>, respectively.

The normally preferred procedure for preparing the monopropellants of the invention is to admix the quaternary ammonium compound, prepared by any suitable method, with nitric acid or other suitable oxidant in the 65 desired ratio at some time prior to use. It is generally preferred to add the quaternary ammonium compound to the acid oxidant at temperatures below about 50° C., e.g. 0 to 30° C., with good agitation. The length of storage prior to use will depend upon the storage stability of the 70 particular monopropellant composition being employed as will be shown hereinafter.

The quaternary ammonium compound-nitric acid monopropellants of the present invention can be conveniently ignited by contacting a stream of the mono- 75 propellant with a stream of a hypergol such as pyrrole.

Any material which is hypergolic when mixed with nitric acid can be used. Other materials hypergolic with nitric acid such as N,N,N',N'-tetramethylpropane-1,3-diamine; N,N,N',N'-tetramethylpropene-1,3-diamine; furfuryl alcohol; ethylenediamine; etc., can also be used to ignite the two-component monopropellant. These hypergols are simultaneously injected into the combustion chamber with the two-component monopropellant to ignite the monopropellant. After the two-component monopropellant is ignited, the flow of hypergol is stopped. A temperature-sensitive element, a time mechanism or other means can be used to terminate the flow of the hypergol. The monopropellant compositions of the present invention can also be ignited by other means such as, for example, by an electric igniter.

The quaternary ammonium compounds used in the practice of the invention can be prepared by any of a number of suitable methods well known to those skilled in the art. A first method, by which the majority of the compounds tested in Example I were prepared, comprises, in general, the addition of a suitable alkyl chloride to a suitable amine which has been dissolved in a highly polar solvent such as nitrobenzene. The choice of the alkyl chloride, the amine, and the specific reaction temperature and quantities of reactants and solvents will of course depend upon the particular compound it is desired to prepare as will be understood by those skilled in the art. Methyl alcohol can be used as a co-solvent to increase the solubility of the alkyl chloride in the polar solvent, if desired. After reaction of said alkyl chloride and said amine, the resulting quaternary ammonium chloride is separated and dried under vacuum. Said quaternary ammonium chloride is then dissolved in methyl alcohol and the exact percent of the chloride salt in solution is determined gravimetrically by means of silver chloride precipitation.

The thus obtained standardized alcoholic quaternary

ammonium chloride solution is then treated with a stoichiometric amount of standardized alcoholic potassium hydroxide solution and the resulting potassium chloride which precipitates (essentially quantitative) is filtered. The filtrate is then treated with approximately a 10% excess of the acid corresponding to the quaternary ammonium salt to be prepared, e.g., nitric acid for nitrates, perchloric acid for perchlorates, etc. After the acid addition is complete, the mixture is evaporated to near dryness on a steam bath. The mushy residue is then dissolved in a minimum amount of isopropyl alcohol and the quaternary ammonium salt precipitates as a white crystalline product upon the addition of ethyl ether. The precipitated quaternary ammonium salt is filtered, washed with more ether and dried in a vacuum desiccator. This procedure has been found reliable and the quaternary ammonium salts so prepared are normally obtained in yields of 90-98 weight percent.

A second method comprises treating a trialkylamine with a solution of an alkyl nitrate in ethyl ether and allowing the mixture to stand for several days, after which the solvent is evaporated. Triethylmethylammonium nitrate was obtained by this procedure in a yield of 5.2 percent of theoretical.

A third method comprises treating a suitable amine with a suitable alkyl halide and then reacting silver nitrate with the resulting quaternary ammonium halide to produce the corresponding quaternary ammonium nitrate. Tetraethylammonium nitrate and triethylmethylammonium nitrate were prepared by this method.

#### EXAMPLE I

Quaternary ammonium compounds prepared by one of the above described procedures were admixed with anhydrous nitric acid at room temperature in stoichiometric proportions. Properties of the mixtures are given below in Table I.

Table I

PROPERTIES OF ANHYDROUS NITRIC ACID-QUATERNARY AMMONIUM COMPOUND MONOPROPELLANTS

|                                                               | Unmixed compound |                    | Stoichiometric mixtures with anhydrous nitric acid |                                                       |                                              |                                                  |                                     |                           |        | Calculated performance |        |                      |                  |
|---------------------------------------------------------------|------------------|--------------------|----------------------------------------------------|-------------------------------------------------------|----------------------------------------------|--------------------------------------------------|-------------------------------------|---------------------------|--------|------------------------|--------|----------------------|------------------|
|                                                               | Molecular weight | Melting point, °C. | Compound content of mixture (weight percent)       | Oxidizer to fuel ratio W <sub>o</sub> /W <sub>s</sub> | Freezing point <sup>1</sup> of solution, °F. | Storage stability, hrs. to 100 p.s.i. at 200° F. | Card gap value (cards) <sup>2</sup> | Density gm./ml. at 20° C. | 75° F. | 32° F.                 | 40° F. | Max. I <sub>ep</sub> | O/F <sup>3</sup> |
| Tetramethylammonium nitrate.                                  | 136.2            | >290               | 32.9                                               | 2.04                                                  | -24                                          | >840                                             | 2-4 gl.                             | 1.396                     | 2.42   | 3.92                   | -----  | 225.2                | 1.455            |
| Tetramethylammonium perchlorate.                              | 174.6            | >290               | 42.0                                               | (a)                                                   | (a)                                          | (a)                                              | (8-16) sat'd soln. gl.              | -----                     | -----  | -----                  | -----  | 228.7                | 0.766            |
| Triethylmethylammonium nitrate.                               | 178.2            | >290               | 26.1                                               | 2.82                                                  | <-94                                         | >838                                             | 8-10 gl.                            | 1.350                     | 1.33   | 1.92                   | 5.18   | 223.2                | 2.020            |
| Triethylmethylammonium perchlorate.                           | 215.7            | >290               | 31.6                                               | 2.17                                                  | <-94                                         | >478                                             | 32-34 gl.                           | 1.374                     | 1.52   | 1.88                   | 4.28   | 225.3                | 1.441            |
| Triethylmethylammonium dihydrogen phosphate.                  | 213.2            | 100-120            | 27.3                                               | 2.67                                                  | <-94                                         | >712                                             | -----                               | -----                     | -----  | -----                  | -----  | -----                | -----            |
| Triethylmethylammonium hydrogen sulfate.                      | 213.3            | 177-187            | 28.2                                               | 2.54                                                  | <-94                                         | >816                                             | -----                               | 1.412                     | 1.95   | 3.17                   | 12.29  | -----                | -----            |
| Tetraethylammonium nitrate.                                   | 192.3            | >290               | 24.9                                               | 3.02                                                  | <-94                                         | 3 750                                            | 30-36 st., 24-26 gl.                | 1.355                     | 1.55   | 1.90                   | 4.61   | 223.8                | 2.154            |
| Tetraethylammonium perchlorate.                               | 229.7            | >290               | 29.8                                               | 2.36                                                  | -80                                          | 3 195                                            | 21-22 gl., 40-42 st.                | 1.420                     | -----  | -----                  | -----  | 225.5                | 1.573            |
| Tetraethylammonium dihydrogen phosphate.                      | 227.3            | 143 and 242        | 26.1                                               | 2.84                                                  | <-94                                         | 72                                               | -----                               | -----                     | -----  | -----                  | -----  | -----                | -----            |
| Tetraethylammonium hydrogen sulfate.                          | 227.3            | >290               | 26.9                                               | 2.72                                                  | <-94                                         | 3 94                                             | -----                               | -----                     | -----  | -----                  | -----  | -----                | -----            |
| Tetra-n-propylammonium nitrate.                               | 248.4            | 260 (dec.)         | 22.0                                               | 3.55                                                  | -64                                          | 360                                              | 60-73 gl., 80-85 st.                | 1.15                      | 1.56   | 3.41                   | 223.7  | 2.537                | -----            |
| Tetra-n-propylammonium perchlorate.                           | 285.8            | 241-244            | 25.3                                               | 2.95                                                  | -56                                          | 38                                               | -----                               | 1.348                     | 1.02   | 1.43                   | 3.35   | 224.6                | 2.110            |
| Tetra-n-propylammonium dihydrogen phosphate.                  | 283.4            | 158-170            | 23.1                                               | 3.34                                                  | <-94                                         | 4 381                                            | -----                               | -----                     | -----  | -----                  | -----  | -----                | -----            |
| Tetra-n-propylammonium hydrogen sulfate.                      | 283.4            | 136-144            | 23.6                                               | 3.24                                                  | -63                                          | 288                                              | -----                               | 1.383                     | 1.29   | 1.97                   | 5.88   | -----                | -----            |
| N,N'-dimethyltriethylene diammonium dinitrate.                | -----            | -----              | 35.6                                               | 1.80                                                  | -43                                          | >912                                             | -----                               | 1.51                      | -----  | -----                  | -----  | -----                | -----            |
| N,N'-diethyltriethylene diammonium dinitrate.                 | -----            | -----              | 31.7                                               | 1.84                                                  | <-94                                         | 3>72                                             | 11-12                               | 1.52                      | -----  | -----                  | -----  | -----                | -----            |
| N,N'-diisopropyltriethylene diammonium dinitrate.             | -----            | -----              | 29.2                                               | 2.38                                                  | <-94                                         | 3>120                                            | -----                               | -----                     | -----  | -----                  | -----  | -----                | -----            |
| N,N,N',N',N',N' - hexamethylmethane-1,2-diammonium dinitrate. | 270.3            | 233d               | 33.8                                               | 1.96                                                  | -58                                          | >1030                                            | >22 st., 12-14 gl.                  | 1.443                     | 5.6    | 11.01                  | 104.6  | 224.8                | 1.399            |

See footnotes at end of table.

Table I—Continued

|                                                                                | Unmixed compound |                     | Stoichiometric mixtures with anhydrous nitric acid |                                           |                                              |                                                  |                                     |                           |                        | Calculated performance |       |                      |                  |
|--------------------------------------------------------------------------------|------------------|---------------------|----------------------------------------------------|-------------------------------------------|----------------------------------------------|--------------------------------------------------|-------------------------------------|---------------------------|------------------------|------------------------|-------|----------------------|------------------|
|                                                                                | Molecular weight | Melting point, °C.  | Compound content of mixture (weight percent)       | Oxidizer to fuel ratio Wa/Ws <sup>6</sup> | Freezing point <sup>1</sup> of solution, °F. | Storage stability, hrs. to 100 p.s.i. at 200° F. | Card gap value (cards) <sup>2</sup> | Density gm./ml. at 20° C. | Viscosity, centistokes |                        |       | Max. I <sub>sp</sub> | O/F <sup>5</sup> |
| N, N, N, N', N', N' - hexamethylethane-1,2-diammonium diperchlorate.           | 345.2            | >290                | 43.0                                               | 1.33                                      | >792                                         |                                                  |                                     | 1.506                     |                        |                        |       | 227.1                | 0.730            |
| N, N, N, N', N', N' - hexamethylethane-1,2-bis(ammonium hydrogen sulfate).     | 340.4            | >290                | 40.3                                               | 1.48                                      | 450                                          |                                                  |                                     | 1.500                     |                        |                        |       |                      |                  |
| N, N, N, N', N', N' - hexamethylethane-1,2-bis(ammonium dihydrogen phosphate). | 340.2            | >290                | 39.2                                               | 1.55                                      | b-85                                         | 792                                              |                                     | 1.516                     |                        |                        |       |                      |                  |
| N,N,N',N',N' - tetramethyldiethylenediammonium dinitrate.                      |                  | >275                | 34.7                                               | 1.88                                      |                                              | >192                                             |                                     | 1.43                      |                        |                        |       |                      |                  |
| N,N,N',N',N' - hexamethylpropane-1,2-diammonium dinitrate.                     | 284.3            | 132-138             | 32.0                                               | 2.12                                      |                                              | 288                                              | 10-11 st.                           | 1.448                     | 5.0                    | 9.75                   | 68.8  | 224.5                | 1.520            |
| N,N,N',N',N' - hexamethylpropane-1,2-bis(ammonium dihydrogen phosphate).       | 359.2            | 204-215             | 40.4                                               | 1.48                                      |                                              | 3>24                                             |                                     | 1.47                      |                        |                        |       | 225.7                | 0.921            |
| N,N,N',N',N' - hexamethylpropane-1,3-diammonium dinitrate.                     | 354.3            | 238-243 and 242-246 | 37.0                                               | 1.70                                      |                                              | 22.7                                             |                                     |                           |                        |                        |       |                      |                  |
| N,N,N',N',N' - hexamethylpropane-1,3-bis(ammonium dihydrogen phosphate).       | 284.3            | >290                | 32.0                                               | 2.13                                      | <-94                                         | >818                                             | 12-16 st., 4-8 gl.                  | 1.423                     | 4.3                    | 8.3                    | 48.1  | 224.5                | 1.520            |
| N,N,N',N',N' - hexamethylpropane-1,3-diammonium dinitrate.                     | 359.2            | >290                | 40.4                                               | 1.48                                      |                                              |                                                  |                                     |                           |                        |                        |       | 225.4                | 0.921            |
| N,N,N',N',N' - hexamethylpropane-1,3-bis(ammonium dihydrogen phosphate).       | 354.3            | 220-225 and 235-241 | 36.9                                               | 1.71                                      |                                              | 792                                              |                                     | 1.47                      | 8.8                    | 23.7                   | 318.1 |                      |                  |
| N,N,N',N',N' - hexamethylpropane-1,3-bis(ammonium dihydrogen phosphate).       | 354.4            | 187-195 and >290    | 36.0                                               | 1.78                                      |                                              | 469                                              |                                     |                           | 7.4                    | 15.9                   | 133.0 |                      |                  |
| N,N,N',N',N' - hexamethylbutane-1,3-diammonium dinitrate.                      | 298.4            | 135-142             | 30.5                                               | 2.28                                      | <-94                                         | >580                                             | 12-14 st., 4-6 gl.                  | 1.424                     | 3.96                   | 7.36                   | 44.3  | 224.2                | 1.629            |
| N,N,N',N',N' - hexamethylbutane-1,3-diammonium dinitrate.                      | 373.2            | >290                | 38.2                                               | 1.62                                      |                                              |                                                  |                                     |                           |                        |                        |       | 226.1                | 1.013            |
| N,N,N',N',N' - hexamethylbutane-1,3-diammonium dinitrate.                      | 368.4            | 246-260             | 35.2                                               | 1.84                                      |                                              | 984                                              |                                     |                           |                        |                        |       |                      |                  |
| N,N,N',N',N' - hexamethylbutane-1,3-bis(ammonium dihydrogen phosphate).        | 368.5            | 206-214 and >290    | 32.8                                               | 2.05                                      |                                              |                                                  |                                     |                           |                        |                        |       |                      |                  |
| N,N,N',N',N' - hexamethylbutane-1,4-diammonium dinitrate.                      | 298.4            | 256-266             | 30.5                                               | 2.28                                      | <-85                                         | >742                                             |                                     | 1.417                     | 3.3                    | 5.7                    | 26.7  | 224.2                | 1.629            |
| N,N,N',N',N' - hexamethylbutane-1,4-diammonium dinitrate.                      | 373.2            | >290                | 38.2                                               | 1.62                                      | <-85                                         | 165                                              |                                     | 1.448                     | 2.8                    | 4.5                    | 16.4  | 226.1                | 1.013            |
| N,N,N',N',N' - hexamethylbutane-1,4-bis(ammonium dihydrogen phosphate).        | 368.5            | 223-231             | 32.8                                               | 2.05                                      | <-85                                         | 3>463                                            |                                     | 1.453                     | 4.9                    | 9.4                    | 48.4  |                      |                  |
| N,N,N',N',N' - hexamethylbutane-1,4-bis(ammonium dihydrogen phosphate).        | 368.3            | 110 and 245         | 31.3                                               | 2.19                                      | <-85                                         | 3>312                                            |                                     | 1.468                     | 5.2                    | 10.8                   | 28.4  |                      |                  |
| N,N,N',N',N' - hexamethylhexane-1,4-diammonium dinitrate.                      | 326.4            | 214-223             | 28.2                                               | 2.55                                      | <-94                                         | 199                                              |                                     | 1.389                     | 2.6                    | 4.7                    | 16.3  | 222.9                | 1.820            |
| N,N,N',N',N' - hexamethylhexane-1,6-diammonium diperchlorate.                  | 401.3            | 263-266             | 34.7                                               | 1.88                                      | <-94                                         | 144                                              |                                     | 1.436                     | 1.6                    | 2.4                    | 7.7   | 224.3                | 1.178            |
| N,N,N',N',N' - hexamethylhexane-1,6-bis(ammonium dihydrogen phosphate).        | 396.5            | >290                | 30.4                                               | 2.29                                      | <-94                                         | 230                                              |                                     | 1.443                     | 3.6                    | 7.5                    | 34.6  |                      |                  |
| N,N,N',N',N' - hexamethylhexane-1,6-bis(ammonium dihydrogen phosphate).        | 396.4            | 182 and 245-254     | 29.3                                               | 2.41                                      | <-94                                         | 186                                              |                                     | 1.483                     | 3.6                    | 7.3                    | 34.6  |                      |                  |
| N,N,N',N',N' - hexamethylethane-1,2-diammonium dinitrate.                      | 354.5            | 98-100              | 26.5                                               | 2.78                                      | <-112                                        | 307                                              | 6-7 gl., 20-21 st.                  | 1.327                     | 1.70                   | 3.39                   | 9.37  | 223.8                | 1.981            |

<sup>1</sup> Temperature at which crystal separation begins.<sup>2</sup> gl.=glass cup; st.=steel cup.<sup>3</sup> Leak developed during sample test.<sup>4</sup> Tested on 30.6 percent salt sample.<sup>5</sup> Oxidizer to fuel ratio.<sup>6</sup> Weight of acid/weight of salt.<sup>a</sup> Does not form stoichiometric solution.<sup>b</sup> Glass at—.

The data given in the above Table I show that the thermal stability of the monopropellants of the invention ranges from 23 hours to more than 1080 hours. The card gap tests show that the monopropellants are resistant to detonation by shock. Freezing points are all below

—24° F. and many are below —94° F., showing that the monopropellants are suitable for use under arctic or high altitude conditions. The viscosities show that the monopropellants can be readily pumped at temperatures at least 75 as low as —40° F.

9  
EXAMPLE II

The excellent thermal stability of the monopropellant compositions of the invention is further illustrated by comparison with other previously known monopropellants. In the comparison given below in Table II the "A" compounds represent quaternary ammonium compounds of the invention and the "B" compounds represent acid salts of amines having analogous substituents. A comparison of the tests on said "A" and "B" compounds shows that the quaternary ammonium compounds are surprisingly more stable than the corresponding acid salts of amines. Said tests were run on stoichiometric mixtures of said compounds "A" and "B" in anhydrous nitric acid.

Table II

| Test No. | Compound                                                    | Weight percent compound in mixture | Storage stability, hrs. at 200° F. |
|----------|-------------------------------------------------------------|------------------------------------|------------------------------------|
| 1A       | N,N,N,N',N',N'-hexamethylbutane-1,4-diammonium perchlorate. | 38.2                               | 165                                |
| 1B       | N,N,N,N'-tetramethylbutane-1,4-diamine perchlorate.         | 43.2                               | 29.2                               |
| 2A       | Triethylmethylammonium nitrate                              | 26.1                               | >838                               |
| 2B       | Triethylamine nitrate                                       | 27.7                               | 216                                |
| 3A       | N,N,N,N',N',N'-hexamethylpropane-1,3-diammonium dinitrate.  | 32.0                               | 818                                |
| 3B       | N,N,N',N'-tetramethylpropane-1,3-diamine dinitrate.         | 36.1                               | 2.5                                |
| 4A       | N,N,N,N',N',N'-hexamethylbutane-1,4-diammonium dinitrate.   | 30.5                               | 742                                |
| 4B       | N,N,N',N'-tetramethylbutane-1,4-diamine dinitrate.          | 33.8                               | 6.8                                |
| 5A       | N,N'-dimethyltriethylene-diammonium dinitrate.              | 35.6                               | 912                                |
| 5B       | Triethylene diamine dinitrate                               | 42.1                               | 4.5                                |

EXAMPLE III

The burning rate at 750 p.s.i.g. pressure was determined for a stoichiometric mixture of anhydrous nitric acid with tetramethylammonium nitrate containing 32.9 weight percent of said nitrate. The equipment employed for the determination of said burning rate consisted of an optical bomb which was designed for the burning of solid propellants. The test was performed by placing 2 milliliters of the propellant mixture in an 8 millimeter glass tube and thereafter placing the tube in the bomb. After closing the bomb and pressuring to the desired pressure with nitrogen, the propellant mixture was ignited by means of a short length of Nichrome resistance wire which was immersed in the surface of the propellant liquid. The time required to burn a finite distance was measured, thus the results are expressed directly in inches per second. The burning rate was 0.02 inch per second at ambient temperature (approximately 70° F.).

The procedures used in carrying out the tests in the above examples are outlined below.

The thermal stability tests were carried out at 200° F. on stoichiometric mixtures of the quaternary ammonium compounds in anhydrous nitric acid. The procedure followed can be summarized as follows. A small glass tube, constructed from 1/4-inch (I.D.) glass pipe which is able to withstand pressure greater than 1000 p.s.i., is filled about two-thirds full (about 6 ml.) with the monopropellant to be tested. This tube is fitted with a safety head containing a rupture disk which will rupture at about 200 p.s.i. pressure. Said small glass bomb is then placed in a constant temperature bath, containing cold water, and is connected to a pressure recorder and to a supply of compressed nitrogen gas. The pressure in said bomb is raised to 110 p.s.i. with nitrogen to check the system for leaks after which the pressure in said bomb is reduced to 20 p.s.i. The temperature in the constant temperature bath, which can be regulated to maintain a temperature of 200° F., is increased and the time at which a temperature of 200° F. is reached is taken as the start of

the test. The test is terminated when the pressure in said bomb exceeds 100 p.s.i. or when the rupture disk is ruptured (the pressure rise is often rapid after 100 p.s.i. is reached). The storage life of the propellant at 200° F. is recorded as the time necessary for the pressure in said bomb to increase from 20 to 100 p.s.i.

The shock sensitivity of the monopropellants was determined by the American Rocket Society's Recommended Card Gap Test No. 1, Committee on Monopropellant Test Methods, July 12, 1955. Basically said test consists of placing a 40 ml. sample of the monopropellant above a 50 gram tetryl booster charge and determining the number of 0.01 inch thick cellulose acetate disks ("cards") which must be inserted between said booster and the monopropellant to prevent detonation of said monopropellant sample. The following minor modifications were made in the procedure.

In some of the tests the apparatus was modified so that the blasting cap can be inserted as the last step before firing. This procedure is felt to be safer and more convenient than connecting the cap into the system in the first step. This change was made by cutting slots in the cardboard coupling and pellet tubes and by cutting a horizontal slot in the cap-support block. This allows the cap to be inserted in a horizontal position next to the tetryl booster after the test sample has been put into the cup. This modification is quite easily made and permits the continued use of original apparatus with the advantage of an additional safety feature.

Instead of using the prescribed steel cup for holding the monopropellant sample, many of the tests were run using a cup made of Pyrex glass pipe. The dimensions of the glass cup corresponded closely with those of the recommended steel cup:

|                   | Glass cup dimensions, inches | Steel cup dimensions, inches |
|-------------------|------------------------------|------------------------------|
| Outside dimension | 1.328                        | 1.315                        |
| Wall thickness    | 0.164                        | 0.133                        |
| Inside dimension  | 1.000                        | 1.049                        |
| Length            | 3                            | 3                            |

The data for the card gap test are herein recorded as a range from the highest number of cards which did not prevent detonation to the lowest number of cards which prevented detonation. The shock stability is inversely related to the card gap range.

The viscosities were determined with a Fenske viscometer following the procedure substantially as stated in ASTM Test D445.

The densities were determined with a Westphal balance. The approximate freezing points were determined by cooling the solution to the temperature at which crystal separation began. Some of the tests were terminated at temperatures above the freezing point in view of the low values.

It is to be realized that the storage stability test at 200° F. is a severe test and the mere fact that some compounds give mixtures which have a relatively low storage stability at 200° F. does not mean that said compounds are not useful in the practice of the invention because, at lower temperatures, mixtures of said compounds with nitric acid do have higher storage stabilities than those shown in Table I and can be used at lower temperatures in those instances where storage stability is of secondary importance.

The calculated performance ( $I_{sp}$ ) values of the monopropellants of the invention were calculated using the following formula and assuming frozen combustion gas com-

position during isentropic expansion of combustion gases in the rocket nozzle.

$$I_{sp} = \sqrt{\frac{2}{g} \left( \frac{K_1}{K_1 - 1} \right) \frac{RT_c}{M} \left[ 1 - \left( \frac{P_e}{P_c} \right) \frac{K_2 - 1}{K_2} \right]}$$

Where:

$K_1$  is the ratio of specific heats ( $C_p/C_v$ ) for the combustion gases at the arithmetic mean (*am*) temperature of  $T_c$  and  $T_e$

$K_2$  is the ratio of specific heats of the combustion gases at the logarithmic mean (*lnm*) temperature of  $T_c$  and  $T_e$

$$T_{am} = \frac{T_c + T_e}{2}$$

$$T_{lnm} = \frac{T_c - T_e}{\ln \frac{T_c}{T_e}}$$

$T_c$  is the combustion temperature (or reaction temperature) in the rocket engine in degrees Rankin

$T_e$  is the temperature of the combustion gases after expansion at the nozzle exit (assuming isentropic, optimum expansion) in degrees Rankin

$P_c$  is the combustion chamber pressure in atmospheres

$P_e$  is the pressure in atmospheres at the nozzle exit

$R$  is the universal gas constant

$g$  is gravitational conversion factor

$$\left[ 32.174 \left( \frac{\text{lb. mass}}{\text{lb. force}} \right) \left( \frac{\text{ft.}}{\text{sec.}^2} \right) \right]$$

$M$  is the average molecular weight of combustion gases at combustion chamber conditions

Since many possible embodiments may be made of this invention without departing from the scope thereof, it is to be understood that all matter herein set forth is to be interpreted as illustrative and not in a limiting sense.

We claim:

1. A monopropellant composition consisting essentially of a mixture of (1) an oxidant selected from the group consisting of nitric acid containing at least about 70 weight percent  $HNO_3$  and mixtures of said nitric acid with perchloric acid wherein said mixtures contain up to about 50 weight percent  $HClO_4$  and not more than about 30 weight percent water, and (2) at least one quaternary ammonium compound characterized by a formula selected from the group consisting of



and



wherein: each  $R$  is selected from the group consisting of alkyl, cycloalkyl, alkenyl, and cycloalkenyl radicals containing from 1 to 8 carbon atoms wherein when more than one carbon atom is present the carbon atom attached to the quaternary nitrogen atom is attached to adjoining carbon atoms by single valence bonds, and said radicals substituted with a substituent selected from the group consisting of nitro, nitroso, and cyano radicals, the total number of said substituents in said  $R$  groups being not greater than one-half the total number of carbon

atoms in said  $R$  groups;  $R'$  is selected from the group consisting of alkylene radicals containing from 1 to 12 carbon atoms, and alkenylene radicals containing from 4 to 12 carbon atoms wherein the carbon atom attached to the quaternary nitrogen atom is attached to adjoining carbon atoms by single valence bonds;  $X$  is an anion selected from the group consisting of nitrate, perchlorate, monohydrogen phosphate, dihydrogen phosphate, hydrogen sulfate, sulfate, hydroxyl, orthoborate, dihydrogen borate, and tetraborate anions;  $a$  and  $b$  are each integers of from 1 to 4, and the product of  $a$  multiplied by the number of quaternary nitrogen atoms is equal to the product of  $b$  multiplied by the valence of said anion  $X$ ; and wherein the ratio of said quaternary ammonium compound to said oxidant is within the range of 0.75 to 1.25 times that of the stoichiometric amount.

2. The monopropellant of claim 1 wherein said quaternary ammonium compound is  $N,N'$ -dimethyltriethyl-enediammonium dinitrate.

3. The monopropellant of claim 1 wherein said quaternary ammonium compound is  $N,N'$ -diethyltriethylammonium dinitrate.

4. The monopropellant of claim 1 wherein said quaternary ammonium compound is  $N$ -ethyl- $N'$ -methyltriethylammonium dinitrate.

5. The monopropellant of claim 1 wherein said quaternary ammonium compound is tetramethylammonium nitrate.

6. The monopropellant of claim 1 wherein said quaternary ammonium compound is tetraethylammonium nitrate.

7. The monopropellant of claim 1 wherein said quaternary ammonium compound is  $N,N,N',N',N',N'$ -hexamethylpropane-1,3-diammonium dinitrate.

8. The monopropellant of claim 1 wherein said quaternary ammonium compound is  $N,N,N',N',N',N'$ -hexamethylbutane-1,3-diammonium dinitrate.

9. In the method for development of thrust by the combustion of a monopropellant in the combustion chamber of a reaction motor, the step comprising injecting into said combustion chamber a mixture of (1) an oxidant selected from the group consisting of nitric acid containing at least 70 weight percent  $HNO_3$  and mixtures of said nitric acid with perchloric acid wherein said mixtures contain up to about 50 weight percent  $HClO_4$  and not more than about 30 weight percent water, and (2) at least one quaternary ammonium compound characterized by a formula selected from the group consisting of



and



65 wherein: each  $R$  is selected from the group consisting of alkyl, cycloalkyl, alkenyl, and cycloalkenyl radicals containing from 1 to 8 carbon atoms wherein when more than one carbon atom is present the carbon atom attached to the quaternary nitrogen atom is attached to adjoining carbon atoms by single valence bonds, and said radicals substituted with a substituent selected from the group consisting of nitro, nitroso, and cyano radicals, the total number of said substituents in said  $R$  groups being not greater than one-half the total number of carbon atoms in said  $R$  groups;  $R'$  is selected from the group

consisting of alkylene radicals containing from 1 to 12 carbon atoms, and alkenylene radicals containing from 4 to 12 carbon atoms wherein the carbon atoms attached to the quaternary nitrogen atom is attached to adjoining carbon atoms by single valence bonds; X is an anion selected from the group consisting of nitrate, perchlorate, monohydrogen phosphate, dihydrogen phosphate, hydrogen sulfate, sulfate, hydroxyl, orthoborate, dihydrogen borate, and tetraborate anions; a and b are each integers of from 1 to 4, and the product of a multiplied by the number of quaternary nitrogen atoms is equal to the product of b multiplied by the valence of said anion X; and wherein the ratio of said quaternary ammonium compound to said oxidant is within the range of 0.75 to 1.25 times that of the stoichiometric amount.

10. The method of claim 9 where said quaternary ammonium compound is N,N'-dimethyltriethylenediammonium dinitrate.

11. The method of claim 9 wherein said quaternary ammonium compound is N,N'-diethyltriethylenediammonium dinitrate.

12. The method of claim 9 wherein said quaternary ammonium compound is N-ethyl-N'-methyltriethylenediammonium dinitrate.

13. The method of claim 9 wherein said quaternary ammonium compound is tetramethylammonium nitrate.

14. The method of claim 9 wherein said quaternary ammonium compound is tetraethylammonium nitrate.

15. The method of claim 9 wherein said quaternary ammonium compound is N,N,N',N'-hexamethylpropane-1,3-diammonium dinitrate.

16. The method of claim 9 wherein said quaternary ammonium compound is N,N,N',N'-hexamethylbutane-1,3-diammonium dinitrate.

No references cited.